

Patented Feb. 9, 1926.

1,572,266

# UNITED STATES PATENT OFFICE.

LEONARD E. BRANCHEN, OF ROCHESTER, NEW YORK, ASSIGNOR TO EASTMAN KODAK COMPANY, OF ROCHESTER, NEW YORK, A CORPORATION OF NEW YORK.

## PROCESS FOR REDUCING THE VISCOSITY CHARACTERISTICS OF NITROCELLULOSE.

No Drawing.

Application filed May 13, 1925. Serial No. 30,082.

To all whom it may concern:

Be it known that I, LEONARD E. BRANCHEN, a citizen of the United States of America, residing at Rochester, in the county of Monroe and State of New York, have invented certain new and useful Improvements in Processes for Reducing the Viscosity Characteristics of Nitrocellulose, of which the following is a full, clear, and exact specification.

This invention relates to processes for reducing the viscosity characteristics of nitrocellulose. One object of the invention is to provide a safe, simple and inexpensive process for reducing said viscosity characteristics within a comparatively short time. Another object of the invention is to provide a process for reducing rapidly and accurately the viscosity characteristics of the nitrocellulose when it is in the solid colloidized state and even when mixed with high-boiling organic compounds. Another object is to provide a process which is successful at atmospheric pressure and room temperature. Another object of the invention is to provide a process in which the nitrocellulose remains substantially undissolved, thereby avoiding unnecessary and troublesome precipitation steps. Other objects will hereinafter appear.

It is highly desirable, when making solutions of nitrocellulose for spraying, to have a high concentration of nitrocellulose and yet to keep the viscosity of the solutions at a low point. In order to obtain such solutions from the nitrocelluloses which have high viscosity characteristics, it is necessary to modify the latter. The kinds of nitrocellulose which are found in pyroxylin waste and film scrap, and similar waste materials, are nearly always of the high-viscosity species. It is, therefore, desirable to provide a suitable process for lowering the viscosity characteristics of nitrocellulose, particularly when the latter is in solid colloidized form, and associated with high-boiling compounds, like camphor and butyl alcohol, in inexpensive or waste materials.

I have found that such a process can be carried out by first softening the nitrocellulosic material with a suitable liquid and thereafter treating it with an aqueous alkaline solution. The softening step, which is carried out preferably by a penetrant liquid, makes the nitrocellulosic material more

readily susceptible to the action of the alkaline solution and thereby shortens the necessary time for producing the desired result. Various penetrant liquids may be employed such, for example, as one which softens the nitrocellulosic material, like films and has a solvent action on high-boiling organic compounds therein like camphor, butyl alcohol, triphenyl phosphate, monochlornaphthalene, and the like. It is sometimes useful to control the action of an especially strong penetrant by diluting it with water; and in any event the softening action is stopped before the nitrocellulose itself is substantially dissolved.

The treatment with an aqueous alkaline solution may be carried out in many different ways; but the simplest is to operate at room temperature and atmospheric pressure. Moreover, it is advantageous to use dilute solutions so that the nitrocellulose will not be deteriorated by saponification. I prefer to employ an aqueous solution of an alkali that supplies less hydroxyl ions than a 5% aqueous solution of sodium hydroxid. In fact, a much weaker solution than that can be employed, such, for example, as one equivalent to a 2% solution of carbonate of soda. When working with dilute solutions the action can be expedited by heating the bath, but this is not necessary for practical results, since the desired effect can usually be obtained at room temperature in about 3 days. The most useful alkalies to use are the carbonates or hydroxids of the alkali metals, by which term I include the ammonium compounds, as well as those of sodium, potassium, lithium, etc.

I have also found that it is a great advantage to have a bleaching agent present in the alkaline bath. It not only decolorizes the nitrocellulose, so as to yield a superior product, but may assist the alkali in bringing about a reduction in the viscosity characteristics. While any of the usual bleaching agents may be employed, I find it sufficient to bubble chlorine gas into the bath, the amount depending upon the needs for bleaching.

I shall now describe one embodiment of my invention, but it will be understood that the latter is not restricted to the illustrative details except as indicated in the appended claims. The material to be treated is preferably comminuted. Solid colloidized nitro-

cellulose, such as pyroxylin waste, or film scrap from which the gelatinous coatings have been removed in the usual way, is chopped up to a suitable size.

5 The comminuted material is then treated by the penetrant liquid, say a bath of methyl alcohol toned down by 5% of water. The material is allowed to soften in contact with this liquid, preferably by being immersed 10 in it, for 1 to 5 hours at room temperature and atmospheric pressure. In any event the action is stopped before the nitrocellulose is substantially dissolved, and before the pieces gum together in an unmanageable mass.

15 This treatment softens the material and leaches out some of the high-boiling organic compounds which are present with the nitrocellulose.

When the material is suitably softened, if 20 is treated, say by immersion, in the alkaline bath. One containing 2% of sodium carbonate in water, with the desired amount of chlorine gas bubbled in to produce a colorless product, is excellent. The viscosity 25 characteristics of the nitrocellulose are usually reduced in such a bath to the desired point in about 3 days at room temperature and atmospheric pressure. The duration of the action can be readily found 30 by test, say by removing representative samples, dissolving them and making the customary viscosity determinations.

When the end point is reached, the bath is drained from the material and the latter is 35 washed in any suitable way, say by treating it for several days in running water, or by giving it a plurality of soakings in successive baths of water. Purification may be hastened by using baths of hot water, say at 40 75° C.

Instead of the mixture of water and methyl alcohol described above, I may employ ordinary denatured ethyl alcohol, of the kind containing a small amount of methyl alcohol. This operates on average nitrocellulosic materials in about 24 hours at room temperature and atmospheric pressure.

The product obtained by the above described process has been found to be especially free from color and from harmful acidity, as well as remarkably stable.

Having thus described my invention, what I claim as new and desire to secure by Letters Patent is:

1. The process of treating nitrocellulose, which comprises first softening it with a penetrant liquid, and thereafter acting on it separately with an aqueous solution of an alkali until the viscosity characteristics of the nitrocellulose are reduced.

2. The process of treating solid colloidized nitrocellulose associated with a high-boiling organic compound, which comprises first softening it with a penetrant liquid, which

has a solvent action on said organic compound, and thereafter acting on said material with an aqueous solution of an alkali until the viscosity characteristics of the nitrocellulose are reduced.

3. The process of treating solid colloidized nitrocellulosic material, which comprises softening it with a penetrant liquid containing water and an active nitrocellulose solvent, stopping the action of said liquid before the nitrocellulose is dissolved, and thereafter acting on it with an aqueous solution of an alkali until the viscosity characteristics of the nitrocellulose are reduced.

4. The process of treating solid colloidized nitrocellulose associated with a high-boiling organic compound, which comprises softening it with a mixture of water and methyl alcohol, and stopping the action before the nitrocellulose is dissolved, and thereafter acting on it with an aqueous solution of an alkali until the viscosity characteristics of the nitrocellulose are reduced.

5. The process of treating solid colloidized nitrocellulose, which comprises acting thereon with a penetrant liquid, from 1 to 24 hours at room temperature, the action being stopped before the nitrocellulose is dissolved, and thereafter acting on it separately with an aqueous solution of an alkali until the viscosity characteristics of the nitrocellulose are reduced.

6. The process of treating solid colloidized nitrocellulose, which comprises softening it with a penetrant liquid, and thereafter acting on it separately with an aqueous solution of an alkali that supplies less hydroxyl ions than a 5% solution of sodium hydroxid, until the viscosity characteristics of the nitrocellulose are reduced.

7. The process of treating solid colloidized nitrocellulose associated with a high-boiling organic compound, which comprises softening it with a penetrant liquid which has a solvent action on said organic compound, and thereafter acting on it with an aqueous solution of an alkali that supplies less hydroxyl ions than a 5% solution of sodium hydroxid, until the viscosity characteristics of the nitrocellulose are reduced.

8. The process of treating solid colloidized nitrocellulose, which comprises softening it with a penetrant liquid, and thereafter acting on it separately with a 2% solution of a carbonate of an alkali metal, until the viscosity characteristics of the nitrocellulose are reduced.

9. The process of treating nitrocellulose, which comprises softening it with a penetrant liquid, and thereafter acting on it separately with an aqueous solution of an alkali and a bleaching agent, until the viscosity characteristics of the nitrocellulose are reduced.

10. The process of treating solid colloid-

ized nitrocellulose associated with a high-boiling organic compound, which comprises softening it with a penetrant liquid which has a solvent action on said organic compound, and thereafter acting on it with an aqueous solution of an alkali that supplies less hydroxyl ions than a 5% solution of sodium hydroxid, said solution containing a bleaching agent, and said action being continued until the viscosity characteristics of the nitrocellulose are reduced.

5 film scrap which comprises softening it with a bath of water and methyl alcohol for 1 to 5 hours at room temperature, the softening being stopped before the nitrocellulose is dissolved, and thereafter acting on said film scrap with a 2% solution of sodium carbonate containing chlorine for 1 to 3 days at room temperature.

10 Signed at Rochester, New York, this 22nd day of April 1925.

15 20

11. The process of treating comminuted

LEONARD E. BRANCHEN.